

# UNITED STATES PATENT OFFICE.

ERNEST ROGERS, OF NEW LEXINGTON, OHIO.

## LIQUID COATING COMPOSITION.

1,244,777.

Specification of Letters Patent. Patented Oct. 30, 1917.

No Drawing.

Application filed May 9, 1916. Serial No. 96,274.

To all whom it may concern:

Be it known that I, ERNEST ROGERS, a citizen of the United States, and resident of New Lexington, in the county of Perry and

5 State of Ohio, have invented a new and useful Improvement in Liquid Coating Compositions; and I do hereby declare the following to be a full, clear, and exact description thereof.

10 My invention relates to a liquid coating composition in the nature of a vehicle or thinner for paint pigments or pulp for wood, brick or other surfaces to which it may be found applicable.

15 Most compositions of this character are, generally speaking, said to consist of pigment and a vehicle filling the space between the pigment particles. It is well-known that linseed oil and equivalent vegetable oils

20 are the essential vehicles of such compositions or paints. For many years the comparatively high price of linseed oil or equivalent vegetable oils has led to attempts to replace them by other oils, but substantially

25 without commercial success. Either the other oils are about as expensive as linseed oil; or they fail to dry in a commercially feasible length of time. Because of the comparative cheapness of petroleum and

30 some of its distillates, attempts have been made to dilute the linseed oil with these materials. When low boiling portions of petroleum were used, they acted merely as temporary diluents or thinners. They evap-

35 orated almost completely when the paint was applied and the result was merely a paint film with insufficient vehicle. When higher boiling or comparatively non-volatile petroleum fractions were used, the paint

40 simply did not dry in a commercially feasible time. This result was naturally attributed on scientific grounds to the so-called "non-drying" character of petroleum. The drying character of linseed oil is commonly

45 attributed to its power of thickening or solidifying upon absorbing oxygen from the atmosphere. Petroleum not having this power to any marked extent, would naturally not "dry" adequately if used as the

50 vehicle of a paint, and could only be used to dilute or adulterate the linseed oil vehicle.

My invention consists in the discovery that crude petroleum of a paraffin base when mixed with a suitable drying mixture

55 may be used to replace linseed oil, in whole or in part, for mixing with pulp or other

pigments for the manufacture of paint, which will dry in a commercially feasible time, or like ordinary linseed or other oil paints.

60 The main constituent of my improved coating composition is crude oil or petroleum of a paraffin base, and this includes not only the oil as taken from deep wells by pumping or natural flow, but includes any 65 kind of mineral oil of a paraffin base, which is taken from the earth, or such oily portions of these materials as may be taken from them by distillation or other treatment, provided the portions selected are not so volatile 70 that they evaporate too readily.

To an oil of this character I add a drying mixture of varying composition and proportions, depending upon the purpose for which the coating composition is to be used. For illustration, I may give the following as a sample of material which will give the desired drying properties; viz:

1 lb. gum camphor dissolved in alcohol, 80 preferably denatured alcohol;

2 lbs. alum in 16 ozs. of hot water;

5 gals. suitable commercial japan or drier.

These ingredients in or about these proportions are added to fifty (50) gallons of 85 petroleum oil of a paraffin base for the making of a lead paint, for instance. It may be here noted that the composition is preferably used cold.

90 The above ingredients are mixed with the oil previously heated to a suitable temperature, but great care should be exercised to avoid fire as boiling over of the mixture may occur.

I do not wish to limit myself in any way to the drier composed of the ingredients as 95 stated above as I wish to include within the scope of my invention any drying mixture, which will combine with a petroleum oil of a paraffin base to form a coating composition with drying properties of the nature required for commercial purposes. Any of the well-known commercial japans may be employed without the addition of the alum and camphor as set forth in the above-described drying mixture.

100 I believe that I am the first to employ a petroleum oil of a paraffin base as a coating composition when accompanied by a suitable drying mixture, which gives the commercial 110 drying results in the substantial absence of linseed or other similar drying or semi-drying oil so-called. I also wish to include

within the scope of my invention any chemical equivalent of the ingredients stated above as composing the drying mixture. By the term "drying mixture" I mean to include 5 any suitable drier in addition to the ordinary commercial japan, which is a well recognized drying mixture.

By the employment of petroleum oil of a paraffin base, I get a coating composition of 10 light color, which is of great advantage where the lighter colors are to be produced; and where it has been used for a stain for shingles or other porous material, it may be employed in the natural state, or suitable 15 coloring matter or pigment may be added to give the desired color effect, as is the common practice in the art when other oils are used as vehicles. Furthermore, my improved composition, when properly colored, may be used as a paint for painting 20 buildings, cars or other structures; or may be even applied to metal, stone or brick.

Vegetable oils, such as linseed, when used 25 as a paint vehicle are a source of weakness as they are subject to decay and damage by chemical rays of sunlight and will not stand sulfur gases. The petroleum vehicle with a

suitable drying mixture would not be subject to these limitations, for by its use I obtain a paint, stain or filler with a mineral vehicle as well as a mineral base, and as most all pigments or coloring matters are mineral, I avoid the decay due to vegetable oils. The composition also holds color better. Within the term "paraffin base petroleum" of the claims, I mean to include distillates as well.

What I claim is:

1. A liquid coating composition containing as its essential constituents a paraffin base petroleum and a drying mixture.

2. A liquid coating composition containing as its essential constituents, a paraffin base petroleum and a drying mixture including camphor dissolved in alcohol and alum in aqueous solution, all combined in substantially the proportions stated.

In testimony whereof I, the said ERNEST ROGERS, have hereunto set my hand.

ERNEST ROGERS.

Witnesses:

OLIE G. BUTT,

THOMAS M. POTTER.